

L. BRADFORD.  
SEPARATION OF MIXED METALLIC SULFIDS.  
APPLICATION FILED OCT. 22, 1914.

1,274,505.

Patented Aug. 6, 1918.



Witnesses:

R. L. Bruck  
H. B. McGill

Inventor,  
Leslie Bradford  
By Hull & Smith  
Atty's.

# UNITED STATES PATENT OFFICE.

LESLIE BRADFORD, OF BROKEN HILL, NEW SOUTH WALES, AUSTRALIA.

## SEPARATION OF MIXED METALLIC SULFIDS.

1,274,505.

Specification of Letters Patent.

Patented Aug. 6, 1918.

Application filed October 22, 1914. Serial No. 868,131.

To all whom it may concern:

Be it known that I, LESLIE BRADFORD, a subject of the King of Great Britain and Ireland, residing at Cummins street, Broken Hill, New South Wales, Australia, have invented new and useful Improvements in the Separation of Mixed Metallic Sulfids, of which the following is a specification.

This invention relates to the treatment of 10 crude oil and slimes containing mixed sulfids, for the preferential separation of lead sulfid or mixed lead and iron sulfids from zinc sulfid; but it is applicable also for the treatment of mixed sulfid ores containing 15 values other than lead and zinc.

Heretofore a variety of processes have been suggested for effecting separation of sulfids from zinc-lead ores by preferential flotation, that is to say, so as to obtain lead 20 sulfid and zinc sulfid more or less separately. Such processes, however, are to a greater or lesser extent, dependent for their effectiveness upon means which take advantage of some inherent characteristic of the sulfids by 25 virtue of which they behave distinctively when submitted to flotation treatment. Such characteristic properties of sulfids are not referable within present knowledge to any very definite causes, but they are exhibited 30 markedly in some ores, such for example as calcitic ores obtained from the Broken Hill mines. It is known that when certain operative conditions are modified to meet the exigencies of particular cases in conducting 35 known methods of flotation, such for instance as "froth" flotation processes, substantially successful preferential flotation of lead sulfid from zinc sulfid is frequently obtainable. These process modifications usually 40 consist in varying the amount and/or the nature of the agitation, or in varying the nature or quantity of the frothing agent employed, or in controlling air supply during agitation. It is also known that it is 45 possible to exalt the flotation effect in respect of lead sulfid by employing mineral water for or by adding certain mineral salts to the water used in operating the flotation process. In all these processes the proportion of the 50 frothing agent used must be controlled with care. If excessive amounts of the frothing agent are used, zinc sulfid is floated up with the lead sulfid. Other causes of partial or total failure have been observed.

55 The present invention consists in an improved process for effecting the preferential

separation of the sulfids from ores or ore products by flotation, its object being to obtain lead sulfid and/or pyrites separately from zinc sulfid, or so that the lead concentrate will contain relatively little zinc and the residual zinc concentrate relatively little lead. The lead sulfid, with the pyrite, if any, is first removed as float concentrate; the blende remains as a residue, which goes 60 down with the gangue, but is subsequently separated therefrom by flotation according to known methods.

The process of preferential flotation separation in which my said invention consists, 70 is distinguished from known processes by the fact that in conducting it the ores or ore products containing the valuable metallic sulfids to be separated are treated in a medium which wets the zinc sulfid, and which 75 does not wet the lead sulfid and/or pyrites and therefore leaves the last named sulfids floatable while rendering the zinc sulfid temporarily immune to flotation. The lead sulfid and/or pyrites are thus obtained first as a 80 float concentrate; thereafter the residues comprising gangue and zinc sulfid are treated for the separation of the zinc sulfid from the gangue.

This "wetting" effect is procured by adding 85 to an acid flotation solution a limited quantity of a substance which is decomposed by said solution and produces in this decomposition a reducing gas which is more or less soluble in the solution. Notably thiosulfates, sulfites and bisulfites are so decomposed in a solution of sulfuric acid with the production of such a gas (sulfur dioxide). With substantially equal result sulfur dioxide 90 may be introduced directly into the solution, 95 either as gas brought into it in a current or added in solution. The like effect is obtained by means of another reducing gas, sulfureted hydrogen, which may be similarly introduced into the solution or may be produced in it by adding sulfids or polysulfids which the solution is capable of decomposing.

In practice a limited quantity of such a reducing agent is introduced into the flotation solution prior to flotation treatment of the ore therein with the object of procuring this zinc "wetting" effect. The reducing agents I prefer to use are those belonging to the first group—viz. thiosulfates 105 sulfites and bisulfites—as I have usually found them more effective than those be-

longing to the second group. I indicate in a later part of this specification certain systematic tests for determining the suitability and effectiveness of reducing agents for 5 the process.

In carrying out the invention the ore or ore products ground to a sufficiently fine state of division to suit requirements are introduced into a return flotation circuit, a 10 small quantity of a suitable reducing agent being first added to the aqueous ore pulp. The pulp is then submitted to flotation separation, preferably a "froth" flotation operation in which an organic or other emulsifying 15 ("frothing") agent and acid are added to the aqueous solution in which the operation is conducted. I find then that the galena and/or pyrites float preferentially and may be recovered substantially by themselves, 20 while the blende remains temporarily immune to flotation because its surface is "wetted" by the active reducing flotation medium. Having thus preferentially removed the galena and/or pyrites, the blende may 25 subsequently be recovered from the residues in any known manner as a high grade zinc concentrate substantially free from galena and/or pyrites. To enable this recovery of zinc to be obtained, the "wetting" effect of 30 the medium used in the separation of the galena and/or pyrites is first corrected by the addition of an oxidizing agent to react with the reducing agent contained in said medium, or by the introduction into the medium of steam and air and the continuous 35 agitation thereof, which answers the same purpose, or by draining the blende and residues from the first operation and then re-submitting the same to any well known 40 flotation operation in a separate circuit of ordinary character.

Sulfuric acid is in practice almost invariably used as the acidifying agent in carrying out the process on account of its effectiveness and cheapness; but any other of the 45 commercial acids will be found more or less effective as a substitute for sulfuric acid.

The quantity of the reducing agent which is required to produce the best effect varies 50 with the nature of the ore, the temperature at which the lead flotation operation is conducted, and also, to some extent, on the quantity of sulfuric acid used in that operation. For these reasons it is not possible 55 to indicate a uniform rule to govern the correct quantity of reducing agent to be used. That quantity must be determined in each case by laboratory tests. Ordinarily from 8 ozs. to 8 lbs. of reducing agent per 60 ton of ore to be treated will be found sufficient for the purpose of my invention, but I do not bind myself strictly to these limits of proportions. The addition of an excessive quantity of reducing agent has a bad 65 effect, in that the preferential flotation of

the galena and/or pyrites is thereby caused to be unduly delayed, the operation taking a longer time to complete. Such excess of reducing agent also renders the subsequent flotation of the blende from the residue more 70 difficult. Insufficiency of reducing agent minimizes the ability of the liquid to wet the zinc sulfid and therefore militates against successful discrimination between lead sulfid and/or pyrites on the one hand 75 and zinc sulfid on the other hand.

The deferred or delayed flotation effect on the zinc sulfid due to the introduction of a reducing agent into the flotation medium, whereby it is caused to be "wetted," varies 80 more or less directly with the proportion of the "wetting" agent in the flotation medium. By varying the proportion of the "wetting" agent used, the flotation of the blende can on the one hand be entirely prevented or 85 substantially so, or on the other hand the blende may be only rendered temporarily immune to flotation for a limited time. A proportion is determined which has the effect of immunizing the zinc sulfid for a sufficient 90 time to enable a satisfactory recovery of the galena contained in the ore prior to submitting the deleaded zincy residue to further flotation for the recovery of the blende.

The process is suitable for the preferential flotation and recovery of galena from coarsely crushed ores as well as from slimes; and is applicable to the treatment of any ore admixture containing galena and/or pyrites and blende irrespective of the proportion of grit and slimes present, so long as the ore particles are of floatable size and have not been subjected to preceding treatment which would render the reducing agent 100 inoperative for the wetting of the zinc sulfid or render the lead sulfid and/or galena 105 non-floatable.

In the actual application of my invention to a Broken Hill mixed sulfid containing zinc and lead sulfids, I conduct the flotation operation in an apparatus such as that shown in sectional elevation in the accompanying drawing. In this drawing *a* is a mixer tank or box provided with a paddle *b* and means such as bevel gearing *c* and *d* 110 for slowly revolving the shaft *b'* so the contents of the tank *a* will be mixed into the condition of a freely flowing pulp. Into this tank or box *a* the pulverized ore and solution are delivered. Near the bottom 115 of the said mixer box *a* is fixed an exit pipe *e* with a valve *f* to regulate the flow of the pulp to a centrifugal pump *g* which in this case is used as an agitator. The runner shaft *g'* of the pump *g* may be driven by the pulley *g<sup>2</sup>* and supported in bearings *g<sup>3</sup>*. The intake pipe *h* to the pump has a small pipe *i* fixed in it for the addition of sulfuric acid 120 in any required quantity. A steam air injector *k* is tapped into the barrel of the 125

5 pump  $g$  for the dual purpose of heating the ore pulp, and for the introduction of atomized air if found necessary. The exit pipe  $l$  from the centrifugal pump is provided with a valve  $m$  for regulating or throttling the delivery of the agitated pulp in any quantity. The thoroughly gassed pulp is delivered by the pump  $g$  under pressure into a spitzkasten  $n$ , where the separation takes place; the sulfids float to the top, and are allowed to flow away as concentrates by chute  $o$  while the residues sink to the bottom and escape through a continuously running plug hole  $p$ .

15 It will be readily understood that the requisite quantity of reagents can be delivered by gravitation or otherwise into the intake pipe  $h$  to effect the reaction needed in the process and also that the steam and  
20 air entering in adjustable quantities will respectively heat and aerate the pulpy mixture to assist the separation aimed at.

In operation the centrifugal pump fulfils the dual function of churning and delivering the pulpy mixture, the stop valves being so adjusted that the throttling by the valve  $m$  will cause the pulpy liquid to be frothed or aerated by the runner of the pump.

The flotation boxes are set in series and the rate of treatment about 25 tons per hour.

No serious difficulty is experienced in correctly proportioning the sodium thiosulfate used (the blonde "wetting" agent) so as to insure the rapid floating off of the galena substantially pure or as a high grade concentrate rich in silver, and to leave the residue in a condition suitable for further flotation treatment for the recovery of the zinc sulfid therefrom.

The flotation treatment is preferably conducted according to the "froth" flotation principle; the procuring of the effect aimed at is dependent upon the presence of a frothing agent in the flotation medium, only when a reducing gas is introduced into the medium; it is not dependent upon the presence of a frothing agent in the flotation medium when a reducing gas is generated in the flotation medium by reaction of a substance introduced into it. In some cases I find that enhanced results are obtained by digesting the ore with sulfuric acid and the reducing agent in a thick pulp prior to subjecting the same to a flotation operation.

By way of example of the working of this process the following test results are quoted.

(1) 500 grams of a weathered Broken Hill dump slime containing zinc 18.2%, lead 15.2%, oxidized lead 4.0%, silver 18.3 ozs. per ton, were introduced into an agitation flotation machine with 2 liters cold water; 1 gram of sodium thiosulfate was first added, and then 5 c. c. of sulfuric acid. This amount of acid was sufficient to render the

ore pulp slightly acid. A frothing agent was then added in a proportion determined by common experience.

79.5 grams of galena was by this means preferentially floated as a high grade lead concentrate rich in silver, and assaying zinc 9.6%, lead 60%, oxidized lead 2.3%, and silver 69 ozs. per ton. After the galena has been so recovered, 0.1 gram of potassium permanganate was added to neutralize the reducing character of the medium, and the blende was then floated, the recovered product yielding 166.5 grams of a good grade zinc concentrate, assaying zinc 46.4%, lead 6.3%, oxidized lead 1.6%, silver 15.7 ozs. per ton. The tailings resulting from this treatment weighed 238 grams, and assayed zinc 2.0%, lead 7.2%, oxidized lead 6.2%, silver 3.7 ozs. per ton. These operations were carried out in normal atmospheric temperatures. 70 75 80 85

(2) 500 grams of a Broken Hill ore containing zinc 15.5%, lead 11.0%, silver 9.9 ozs. per ton was crushed in a tube mill to a floatable size. The crushed ore consisting of grit and slimes admixed was treated as in the previous test, 0.5 gram of sodium thiosulfate being used, and the operation conducted at a temperature of 100° F. The float of 61 grams of lead concentrates recovered assayed zinc 10.6%, lead 62.8%, silver 35.8 ozs. per ton. After the lead sulfid had been thus preferentially floated, the agitation was continued for a time and a little more acid and frothing agent were added, and 125.5 grams of zinc concentrates were floated. This product assayed, zinc 48.6%, lead 5.8%, silver 15.4 ozs. per ton. The tailings weighed 298.5 grams and assayed zinc 2.8%, lead 2.7%, and silver 2.5 ozs. per ton.

(3) 500 grams of mixed pyrites-blende ore, assaying zinc 28.3%, was introduced into an agitation flotation machine with hot water at a temperature of 140° F. Sufficient sulfuric acid was added to slightly acidify the ore pulp, and then 120 c. c. of a sulfurous acid solution (containing 5 grams sulfurous acid per 100 c. c.) and a sufficiency of a frothing agent were added. 148 grams of pyritic concentrates floated preferentially; these assayed 13.4% zinc. The pulp was then transferred from the flotation machine to a bucket in which the ore was allowed to settle. The supernatant liquor was then decanted, and the ore was reintroduced into the machine, and the blende was floated in hot water to which more frothing agent was added. The zinc concentrates thus floated weighed 220 grams, and assayed zinc 51.6%. The residual tailings weighed 120 grams, and assayed zinc 3.7%. 110 115 120 125

(4) 500 grams of a Tasmanian ore containing a mixture of galena, pyrite, and blende, assaying zinc 28.5%, lead 8.2%, sil- 130

ver 9.5 ozs. per ton, were introduced into a 1000 c. c. stoppered cylinder with 500 c. c. hot water; sulfuric acid was added in sufficient quantity to render the ore pulp slightly acid; and then 2 grams of sodium sulfite were introduced, and the mass was agitated and allowed to stand for 15 minutes. The pulp was then transferred from the cylinder to a floatation machine, and the galena and pyrite were floated preferentially without the addition of any frothing agents at a temperature of 120 deg. F, yielding 200 grams of a mixed pyrite-galena concentrate, assaying zinc 14.2%, lead 13.2%, silver 18.6 ozs. After these products had been preferentially recovered, agitation was continued, a few crystals of potassium permanganate, and a few drops of eucalyptus oil being added. This produced a flotation of 210 grams of zinc concentrates, assaying zinc 53.2%, lead 6.0%, silver 4.0 ozs. The tailings weighed 75 grams and assayed zinc 1.4%, lead 1.0%, silver 1.0 ozs. per ton.

I have not determined all the reducing agents other than sodium thiosulfate and sulfuric acid and sulfurated hydrogen and alkaline sulfites and bisulfites which will operate at suitable, bende "wetting" agents or media for effecting the purpose of this invention. The following described laboratory tests will however satisfactorily determine the efficacy for such purpose of any substance having a reducing action:—

Take 100 grams of the ore to be concentrated in a finely crushed condition. Transfer this ore into a 500 c. c. stoppered cylinder with water. Introduce the "wetting agent" to be tried out, and agitate. Then add sufficient sulfuric acid to render the whole slightly acid. Add a small quantity of a "frothing agent", such as eucalyptus oil, and agitate violently for from two to five minutes. Then critically inspect the contents of the cylinder. If the bende wetting agent employed in the particular test is found to leave the bende particles free and non-granulated, and at the same time permits the galena and/or pyrites particles to granulate or coalesce together, it is an indication that that wetting agent will be found suitable for the treatment of that ore. If the test is made by adding a minimum amount of bende "wetting" agent, and no differentiation is observable between the bende particles on the one hand considered as a group and the galena and/or pyrites particles on the other hand considered as a separate group, repeat the test with a practical maximum quantity of the proposed bende "wetting" agent, and note the difference in behavior of the zinc sulfid from the other sulfids present.

To determine the proper quantity of any particular reducing (bende "wetting") agent to be used for the purpose of this in-

vention to yield the most effective result, and also to ascertain the degree of temperature best suited in particular cases, actual flotation separations must be made on a laboratory scale by first floating the galena and/or pyrites with acidulated solutions containing a predetermined test proportion of the reducing reagent, then draining the remainder of the ore, floating the bende therefrom by known flotation methods, and assaying the floated products in the usual manner. Repe- 70 titions of this test may be made through a range of temperatures and with various percentages of bende "wetting" agent in the first flotation medium.

The particular operative apparatus and manipulations usable for carrying out any flotation operating by means of my herein described process and practically effecting thereby flotation of galena and/or pyrite, 85 are not elements of my invention, and I make no claim upon same. My invention may be successfully carried out by following any well known methods of separating ore products by flotation in known apparatus, and it involves, *qua* flotation apparatus and operations, no novelty.

What I claim as my invention and desire to secure by Letters Patent is:—

1. The process for treating zinc sulfid (bende) ores for the separation of lead sulfid (galena) and pyrite therefrom, which consists in submitting such ores in a more or less finely divided condition to flotation treatment in a separating medium 100 which does not chemically or otherwise permanently affect any of the particles, but does act upon the surfaces of said zinc sulfid (bende) particles by wetting them but without similarly wetting the sulfids mixed therewith, whereby the said zinc sulfid (bende) particles are caused to sink while the remaining sulfids are permitted to float; said separating medium being acidulated water containing in solution a reducing gas 110 containing sulfur.

2. The process for separating zinc sulfid (bende) from admixture with other sulfids such as lead sulfid (galena) and iron sulfids (pyrite), which consists in introducing 115 such sulfid mixture in more or less finely divided condition into an acidulated liquid containing in solution a reducing gas containing sulfur and subjecting the mixture to flotation treatment, whereby said zinc sulfid (bende) particles are wetted and caused to sink and the remaining sulfids permitted to float, decanting said floating sulfids, and afterward reclaiming said zinc sulfid (bende).

3. The process of separating the sulfids of zinc, lead, and iron by selective flotation, which consists in introducing the mixed sulfids into a floating liquid and impregnating the floating liquid with a partially solu- 131

ble reducing gas containing sulfur in quantity sufficient to cause wetting of the sulfid of zinc without affecting the sulfid of lead.

4. The process of separating the sulfids of zinc (blende) from the sulfid of lead (galena) and iron (pyrite) which comprises the step of introducing the comminuted sulfids into a frothing liquid containing a partially soluble sulfurous reducing gas, there-  
10 by causing the wetting of the blende without affecting the galena and without caus-  
ing permanent change on either.

5. The process of separating zinc sulfid (blende) from the sulfids of lead (galena) and iron (pyrite), which consists in submit-  
15 ting such ores in a more or less finely divided condition to flotation in a separating medium which does not chemically or otherwise permanently affect the zinc sulfid (blende) particles, but does act upon the surfaces of said zinc sulfid (blende) par-  
20 ticles by wetting them, whereby the said zinc sulfid (blende) particles are caused to sink while the remaining sulfid particles  
25 are permitted to float, said separating medium being water containing a frothing agent and a soluble reducing gas containing sulfur.

6. The process for separating zinc sulfid (blende) from admixture with other sulfids such as lead sulfid (galena) and iron sulfids (pyrite), which consists in introduc-  
30 ing such sulfid mixture in more or less finely divided condition into an aqueous liquid  
35 containing a frothing agent and a slightly soluble, sulfur-containing, reducing gas, whereby the zinc sulfid (blende) particles are wetted and caused to sink, frothing the liquid, removing the froth-borne sulfids, and  
40 separately recovering the deposited zinc sulfid or blende.

7. In the process of separating the sulfids of zinc, lead, and iron by selective flotation, the step which consists in frothing the sulfids in an aqueous liquid containing in solu-  
45 tion a reducing gas containing sulfur thereby causing the wetting of the sulfid of zinc without affecting the sulfid of lead and without causing chemical change on either.

50 8. The process for treating zinc sulfid (blende) ores for the separation of lead sulfid (galena) and pyrite therefrom, which consists in submitting such ores to flotation in a more or less finely divided condition  
55 in a separating medium which does not chemically or otherwise permanently affect any of the particles, but does act upon the surfaces of said zinc sulfid (blende) par-  
60 ticles by wetting them but without similarly wetting the sulfids mixed therewith, whereby the said zinc sulfid (blende) par-  
65 ticles are caused to sink while the remaining sulfids are permitted to float; said separating medium being water acidulated with sulfuric acid and abounding in sulfur dioxid.

9. The process of separating the sulfids of zinc, lead and iron by selective flotation which comprises the steps of impregnating the floating liquid with sulfur dioxid, intro-  
70 ducing the mixed sulfids therein, and sub-  
jecting them to flotation treatment therein, thereby causing the wetting of the sulfid of zinc without affecting the other sulfids.

10. The process of separating the sulfids of zinc, lead and iron by selective flotation which comprises the steps of acidulating water with sulfuric acid, adding thereto a substance that will react therewith to evolve sulfur dioxid introducing the sulfids in the medium thus formed as a floating liquid, and subjecting the mixed sulfids to flotation treatment therein, said sulfid of zinc being thereby wetted and temporarily rendered immune to flotation without affecting the sulfid of lead.

85 11. The process of separating the sulfid of zinc (blende) from the sulfids of lead (galena) and iron (pyrite) which comprises the step of introducing the comminuted sulfids into a frothing liquid containing an acid and a substance that will react with such acid to evolve a sulfur-containing reducing gas, and submitting said mixed sulfids to flotation treatment therein, said reducing medium causing the wetting of the sulfid of zinc without affecting the sulfid of lead.

12. The process of separating blende from galena and pyrite contained in mixed sulfid ores, which consists in submitting said ores in a finely divided condition to flotation sep-  
10 aration in a medium consisting of a dilute aqueous solution of sulfurous acid, said me-  
dium causing the wetting of the sulfid of zinc and rendering the same temporarily immune to flotation, agitating the mass and  
105 removing the float and sedimentary deposit separately.

13. The process of recovering zinc sulfid (blende) from an ore comprising blende, galena, pyrite, and gangue which consists of submitting the comminuted ore to flotation treatment in an acidulated, aqueous ele-  
110 ment containing a sulfurous reducing gas, whereby the blende and gangue will be caused to sink and the remaining sulfids to float, and thereafter neutralizing the reduc-  
115 ing character and repeating the flotation whereby the blende may be caused to float and the gangue alone to settle.

14. In the process of recovering blende from a compound sulfid ore containing iron, lead, and gangue by the successive flotation method, the steps which consist in first sub-  
120 mitting the comminuted ore to flotation treatment in a floating liquid containing a sulfurous reducing gas, whereby the blende and gangue are wetted and caused to sink, then adding a chemical to neutralize the blende wetting character of the liquid, and finally repeating the floating operation,

whereby the blende is floated away and the gangue deposited.

15. The process of recovering zinc sulfid (blende) from an ore comprising blende, 5 galena, pyrite, and gangue which consists of submitting the comminuted ore to flotation treatment in an aqueous acidulated liquid along with a sulfur-containing chemical of a nature to react with said liquid to 10 produce a soluble, sulfurous, reducing gas, recovering separately the floating and sedimenting parts of the ore, and repeating the flotation of the sedimenting parts with the use of non-reducing liquid.

15 16. The process of flotation consisting in treating ore containing lead and zinc sulfids to divest the zinc sulfid particles of the gaseous envelop about the same, without otherwise altering said zinc sulfid particles, and 20 without removing the envelops of other sulfids, and subjecting the so treated ore to flotation.

17. The process of flotation consisting in so treating ore pulp containing zinc and lead 25 sulfids as to alter the physical conditions at the surfaces of the zinc sulfid particles to render the same immune to the normal adhesion of flotative agents, without chemical alteration of said surface and without similarly affecting the other sulfids, and subjecting 30 the so treated pulp to flotation.

18. The process of separation consisting in delivering ore containing mixed sulfids

to an acidulated bath containing in solution a reducing gas containing sulfur in quantity 35 sufficient to cause wetting of one sulfid without affecting another and without causing chemical change on either, and subjecting the mixture to gas flotation to float the unaffected sulfid.

19. The process of separation consisting in delivering ore containing mixed sulfids to an acidulated bath containing in solution a reducing gas containing sulfur in quantity 45 sufficient to cause wetting of one sulfid without affecting another and without causing chemical change on either, and subjecting the mixture to flotation to float the unaffected sulfid.

20. The process of separation consisting in delivering ore containing mixed sulfids of zinc and lead to an acidulated bath containing in solution a reducing gas containing sulfur in quantity sufficient to cause wetting of the sulfid of zinc without affecting the sulfid of lead and without causing chemical change on either sulfid, and subjecting the mixture to flotation to float the unaffected sulfid.

In testimony whereof I have signed my 60 name to this specification in the presence of two subscribing witnesses.

LESLIE BRADFORD.

Witnesses:

WILLIAM BURBON MARSHALL,  
ARTHUR JAMES LEYSON.